# EUROPEAN PATENT SPECIFICATION

(11) **EP 0 867 530 B1**
(45) Date of publication and mention of the grant of the patent: **07.06.2000**
(21) Application number: 97301617.3
(22) Date of filing: 11.03.1997
(51) Int. Cl.: C25D 11/04, C25D 11/26

(54) **Process and apparatus for coating metals**
Verfahren und Gegenstand für die Beschichtung von Metallen
Procédé and dispositif pour le revêtement des métaux

(43) Date of publication of application: 30.09.1998
(73) Proprietor: Almag AL, Givat Shaul, Jerusalem (IL)
(72) Inventor: Hiterer, Misha, Jerusalem 97854 (IL); Samsonov, Victor, Jerusalem 93805 (IL)
(74) Representative: Lowther, Deborah Jane

(56) References cited:
- EP-A- 0 545 230
- DE-A- 4 104 847
- US-A- 4 668 347

## Description

The present invention relates to a ceramic coating process for valve metals, to articles coated thereby, and to an apparatus for carrying out said process.

Valve metals exhibit electrolytic rectification, and the present invention is therefore concerned with providing a coating process and apparatus for coating aluminium, zirconium, titanium, hafnium, and alloys thereof.

More particularly, the present invention is concerned with an electrolytical process using a shaped-wave, high-voltage alternating current to achieve melting during coating of even a thick layer, such a thick layer being achieved in a short time by changing electrolyte composition during the course of the process.

Aluminium, titanium and their alloys have favourable strength/weight ratios which suit these metals to many applications, for example, for use in aircraft and for fast- moving parts in internal combustion engines. As these metals do not, however, exhibit particularly good wear properties, coatings are often used to improve wear and erosion-resistance. The applied coatings are likely to achieve further design requirements such as resistance to chemicals, particularly acids and alkalies; allowance of exposure to higher temperatures; reduction of friction, and the provision of dielectric properties. While the low-cost, widely-used anodizing process achieves some of these aims for moderate service, ceramic coatings are required for severe service requirements.

A number of electrolytic coating processes for these metals are known, which use direct current and/or voltages below 600 V. Such processes are described, for example, in U.S. Patents 3,956,080; 4,082,626 and 4,659,440. These and the majority of recent disclosures describe processes which form ceramic films using an anode spark discharge technique, and which achieve good results regarding coating corrosion resistance and adhesion. Such methods do, however, have two important drawbacks: low film hardness and slow film formation.

In U.S. Patent 5,147,515, Haganata *et al*. disclose the use in an electrolytic bath of a dispersion comprising an aqueous solution of a water-soluble or colloidal silicate and/or an oxyacid salt to which ceramic particles are dispersed. Voltage is increased during film formation from 50-200 V, and may finally exceed 1000 V. With regard to wave form, said patent states that the output from a power supply may be a direct current having any wave form, but preferably those having a pulse shape (rectangular wave form), saw-tooth wave form, or DC half-wave form. Such language does not imply recognition that a sharply-peaked wave form makes a major contribution to providing a dense, hard film.

The speed of film formation reported in the eight examples provided in said patent can be calculated as follows:

| **Example No.** | **Film Thickness µm** | **Coating Time Minutes** | **Formation Velocity µm/Minute** |
|---|---|---|---|
| 1 | 35 | 20 | 1.75 |
| 2 | 31 | 20 | 1.55 |
| 3 | 28 | 30 | 0.93 |
| 4 | 27 | 20 | 1.35 |
| 5 | 36 | 30 | 1.20 |
| 6 | 14 | 30 | 0.47 |
| 7 | 15 | 30 | 0.50 |
| 8 | 28 | 30 | 0.93 |

Such slow rates of film formation do not compare well with those of the present invention.

Also, no indication was given in U.S. Patent 5,147,515 whether it is possible, through the method of said patent, to produce very thick coatings, e.g., in the range of 300-700 µm.

A recently-developed coating method, known as the Kepla-Coat Process, is based on plasmachemical anodic oxidation. The cathode is the surface film of an organic electrolyte, above which the part to be coated is suspended, forming the anode. A plasma is formed which causes the production of a ceramic coating on the anode and heating of the workpiece. Due to the formation of an oxide film on the anode, the process produces a film no thicker than about 10 µm and terminates in 8-10 minutes. Workpiece heating occurs, as the workpiece is not surrounded by liquid; non-symmetrical or slender workpieces are likely to suffer distortion. A further disadvantage of the Kepla-Coat Process is that the high rate of electrolyte evaporation poses an environmental problem.

It is therefore one of the objects of the present invention to obviate the disadvantages of the prior art ceramic coating processes and to provide a process which produces a hard film with strong adherence and minimum porosity.

It is a further object of the present invention to provide a method for producing coatings up to 300 and more microns thick, within a moderate time span.

The present invention achieves the above objectives and others by providing a process for forming a ceramic coating on a valve metal selected from the group consisting of aluminium, zirconium, titanium, hafnium and alloys of these metals, said process comprising immersing said metal as an electrode in an electrolytic bath comprising an aqueous solution of an alkali metal hydroxide, providing an opposite electrode immersed in or containing the electrolyte liquid, passing a modified shaped-wave alternate electric current from a high voltage source of at least 700 V through a surface of said metal to be coated and said opposite electrode, wherein said modified shaped-wave electric current rises from zero to its maximum height and falls to below 40% of its maximum height within less than a quarter of a full alternating cycle, thereby causing dielectric breakdown, heating, melting, and thermal compacting of a hydroxide film formed on the surface of said metal to form and weld a ceramic coating to said metal, and changing the composition of said electrolyte while said ceramic coating is being formed, said change being effected by adding an oxyacid salt of an alkali metal.

A still further object of the present invention is to provide an apparatus for carrying out the above process in a cost-effective manner. The invention thus provides an apparatus for the batch ceramic coating of articles made of a valve metal selected from the group consisting of aluminium, zirconium, titanium, hafnium and alloys of these metals, said apparatus comprising an electrolytic bath comprising an aqueous solution of an alkali metal hydroxide, an electrode immersed in or containing the electrolyte liquid, another electrode comprising at least one of said articles to be coated and means to suspend said article in said electrolyte, a source of alternate electric current from a high voltage source of at least 700 V, means for shaping the AC wave form whereby shaped wave electric current rises from zero to its maximum height and falls to below 40% of its maximum height within less than a quarter of a full alternating cycle, connector elements to complete an electrochemical circuit, and means for adding to said bath, while the apparatus is in operation, a controlled supply of an oxyacid salt of an alkali metal.

A distinguishing feature of the process of the present invention is its suitability to the production of hard coatings as thick as 300 µm within a reasonable time frame of about 90 minutes. This fast coating rate is achieved by changing the composition of the electrolyte while the coating process is in operation. Coating quality is not compromised by the fast formation of a thick coating, as the modified shaped current achieves momentary melting of the layer near the metal workpiece even after the film has built up to the stated thickness.

The invention will now be described in connection with certain preferred embodiments with reference to the following illustrative figures so that it may be more fully understood.

With specific reference now to the figures in detail, it is stressed that the particulars shown are by way of example and for purposes of illustrative discussion of the preferred embodiments of the present invention only, and are presented in the cause of providing what is believed to be the most useful and readily understood description of the principles and conceptual aspects of the invention. In this regard, no attempt is made to show structural details of the invention in more detail than is necessary for a fundamental understanding of the invention, the description taken with the drawings making apparent to those skilled in the art how the several forms of the invention may be embodied in practice.

In the drawings:
Fig. 1 shows a preferred type of shaped-wave pulse;
Fig. 2 depicts the relationship between coating thickness and electrolysis time;
Fig. 3 is a schematic view of an apparatus for batch coating, and
Fig. 4 is a schematic view of an apparatus for series coating.

The process of the invention will now be described. The process is used to form a ceramic coating on aluminium, zirconium, titanium, and hafnium. The process is also suited to alloys of these metals, provided the total of all alloying elements does not constitute more than approximately 20% of the whole. Process parameters may be optimized to suit the paticular metal being coated and the particular properties of the coating considered important to a specific application.

The metal workpiece to be coated is connected as the electrode of an electrolytic bath and is immersed therein.

For coating aluminium, the bath comprises water and a solution of an alkali metal hydroxide. In an embodiment of the bath where it is required to optimize the coating to provide maximum adhesion between the metal and its coating, the electrolyte consists essentially of an aqueous solution containing between 0.5 to 2 g/liter of sodium hydroxide or potassium hydroxide. Fine particles of various substances are added if it is required to improve the special, for example, low friction, properties of the coating. Where such particles are added, the electrolyte is agitated to keep the particles in suspension. Similarly, coloured coatings are produced by adding fine particles of pigmenting substances.

The preferred opposite electrode for the process is a stainless steel bath containing the electrolyte liquid. Where it is preferred to hold the electrolyte in a non-conducting container, for example, for safety considerations, the electrode from iron, nickel or stainless steel is inserted into the bath in the conventional manner.

A modified shaped-wave alternate electric current from a high voltage source of at least 700 V, typically 800 V for aluminium workpieces, is then passed between the metal workpiece and the other electrode. This results in dielectric breakdown, heating, melting and thermal compacting of a hydroxide film formed on the surface of the metal to form and weld a ceramic coating thereto. The arc microwelding is visible during coating. A convenient and moderate-cost method of obtaining the required shaped-wave electric pulse current is by use of a capacitor bank connected in series between the high voltage source from 800 to 1,000 V and said metal workpiece which is being coated.

Referring now to Fig. 1, there is seen a wave form of preferred shape of current. The effect of using alternating current in combination with a high voltage is to prolong the life of the microarc, which causes intense, local, temporary heating, and as a result, the welding and melting of the coating being formed on the submerged metal workpiece. Anodizing is effected during the first positive half-cycle, the metal workpiece being the positive electrode. Thereafter, the dielectric coating already formed fails dielectrically, thereby starting the generation of microarcs. Arc lifetime extends almost to the end of the first half-cycle. Burning of arc is repeated during the second half-cycle, when the workpiece becomes the negative electrode.

Referring now to Fig. 2, there are seen time/coating thickness relationships for processes wherein electrolyte composition is held constant, designated traces 1 to 5. Trace 1 refers to a process wherein the electrolyte is pure potassium hydroxide. Traces 2 to 5 refer to processes wherein increasing concentrations of sodium tetrasilicate were used.

Trace 6 refers to the process of the present invention. It has been found that much faster coating is made possible by changing the composition of the electrolyte while the ceramic coating is being formed. The change effected comprises adding to the electrolyte a salt containing a cation of an alkali metal and an oxyacidic anion of an element selected from the group comprising B, Al, Si, Ge, Sn, Pb, As, Sb, Bi, Se, Te, P, Ti, Zr, V, Nb, Ta, Cr, Mo, W, Mn and Fe, said salt being added in a concentration of between 2 and 200 g/liter of solution. A preferred element is silicone, and a preferred added salt is sodium tetrasilicate.

As is seen in the graph, changing of the electrolyte composition during operation allows production of a 200-µm thick coating in approximately 50 minutes, indicating a film formation velocity of 4 µm/minute. Tests have shown that this fast film formation is achieved without sacrificing the quality of film adhesion to the metal workpiece.

Obviously, once the added salt has been mixed into the electrolyte, the only practical way of again reducing salt concentration for coating the next batch of metal articles is to add considerable quantities of new electrolyte liquid. This problem is solved, however, in the apparatus to be described further below with reference to Fig. 3.

It has also been found that it is possible to produce a pore-free coating by gradual reduction of the current flow when the film has almost reached its desired thickness. In practice, this is effected by progressively reducing the capacitance used to shape the wave form, thus weakening the current until the process stops.

As will be realized from the above description, the term 'modified' as used herein refers to the fact that the wave form is other than the standard sinosidal form normally associated with a wave of alternating current and is instead modified, e.g., as illustrated in Fig. 1, to optimize the coating effect.

Reference is now made to Table 1, which lists various types of coatings for different requirements. Examples are listed of aluminium alloys which have been ceramically coated to achieve various design requirements. Examples 3 and 4 were produced by the technique described above.

The aluminium alloy known as 'Duralumin' has an alloy designation of 2014 and, because of its strength/weight ratio, has found extensive use in aircraft construction. This alloy was therefore chosen for test coating. Table 2 lists characteristics of an achieved coating and the results obtained.

The invention also provides a ceramically-coated metal article produced by the described process. One example of such an article is an aluminium alloy piston for an internal combustion engine. A second example is an aluminium engine block for an internal combustion engine, intended to operate with minimal lubrication. A third example is a protective tile for spacecraft, designed to survive re-entry into the atmosphere. A fourth example is electric insulation serving also as a heat sink of an electronic board.

Fig. 3 illustrates an apparatus 10 for the batch ceramic coating of articles 12 (first electrode) made of a valve metal selected from the group consisting of aluminium, zirconium, titanium, hafnium and alloys thereof. The apparatus 10 has an electrolytic 40-liter bath 14, comprising an electrolyte liquid 16 of water and a solution of an alkali metal hydroxide. Bath 14 is made of stainless steel and forms the second electrode. Agitation means 15 are provided to stir the electrolyte.

The first electrode comprises at least one of the articles 12 to be coated, and conducting means 18 to suspend said article in the electrolyte liquid 16.

A source of alternate electric current of at least 700 V is a 40,000 V-amp step-up transformer 20, designed to supply up to 800, 900, or 1000 V.

The capacitor bank 22 has a total capacitance of 375 µF and it consists of capacitors with nominal capacitance of 25, 50, 100 and 200 µF. Alternatively, such means could be a rectifier and converter circuit (not shown), or other means of the type shown in Fink and Beaty, The Standard Handbook for Electrical Engineers, 12th Ed., pp. 22-96, 22-97.

Connector elements 24 are also provided to complete an electrochemical circuit. An operator control panel 26 is seen at the left of bath 14, the latter being enclosed behind safety doors 28. The opening of safety doors 28 cuts off the electric power.

A salt-containing feed hopper 30, having a solenoid- operated feed valve 32, provides means for adding salt 34 to bath 14 while the apparatus 10 is in operation. Hopper 30 holds a supply of a salt 34, containing a cation of an alkali metal and an oxyacidic anion of an amorphous element. A suitable salt 34 is sodium tetrasilicate.

Shown in Fig. 4 is apparatus 36 for serial ceramic coating of articles 12. A first electrolytic bath 38 contains electrolyte liquid 16, comprising water and a solution of an alkali metal hydroxide. A second electrolytic bath 40 contains an electrolyte liquid 42, comprising water, a solution of an alkali metal hydroxide, and a low concentration of salt 34. A third electrolytic bath 44 contains an electrolyte liquid 46, comprising water, a solution of an alkali metal hydroxide, and a higher salt concentration than in electrolyte 42.

For convenience, baths 38, 40, 44 can comprise a single stainless steel container 48, provided with two vertical dividers 50, forming the electrode. The other electrode comprises at least one of articles 12 to be coated and conducting means 18, which sequentially suspend article 12 in electrolyte liquids 16, 42, 46. Manual or automatic manipulation means 52 allow the transfer of article 12 from the first bath 38 to the second bath 40, and thence to third bath 44.

In apparatus 36, the electrolyte in each bath remains substantially unchanged during operation, and may therefore be used repeatedly. The use of several electrolytes, each having a different composition, enables coating at speeds of about 2.5-4 µm per minute.

The electrical components used are the same as those described hereinabove with reference to Fig. 3.

It will be evident to those skilled in the art that the invention is not limited to the details of the foregoing illustrated embodiments and that the present invention may be embodied in other specific forms without departing from the essential attributes thereof. The present embodiments are therefore to be considered in all respects as illustrative and not restrictive, the scope of the invention being indicated by the appended claims rather than by the foregoing description.

## Claims

1. A process for forming a ceramic coating on a valve metal selected from the group consisting of aluminium, zirconium, titanium, hafnium and alloys of these metals, said process comprising:
immersing said metal as an electrode in an electrolytic bath comprising an aqueous solution of an alkali metal hydroxide;
providing an opposite electrode immersed in or containing the electrolyte liquid;
passing a modified shaped-wave alternate electric current from a high voltage source of at least 700 V through a surface of said metal to be coated and said opposite electrode, wherein said modified shaped-wave electric current rises from zero to its maximum height and falls to below 40% of its maximum height within less than a quarter of a full alternating cycle, thereby causing dielectric breakdown, heating, melting, and thermal compacting of a hydroxide film formed on the surface of said metal to form and weld a ceramic coating to said metal, and
changing the composition of said electrolyte while said ceramic coating is being formed, said change being effected by adding an oxyacid salt of an alkali metal.

2. The process as claimed in claim 1, wherein said modified shaped-wave electric current is obtained by use of a capacitor bank connected in series between said high voltage source and said metal.

3. The process as claimed in claim 1 or claim 2, wherein said added salt is sodium tetrasilicate.

4. The process as claimed in any previous claim, optimized to provide maximum adhesion between said metal and said coating, wherein said electrolyte consists essentially of an aqueous solution containing between 0.5-2 g/liter of sodium hydroxide.

5. The process as claimed in any previous claim, optimized to provide maximum adhesion between said metal and said coating, wherein said electrolyte consists essentially of an aqueous solution containing between 0.5-2 grams per liter of potassium hydroxide.

6. The process as claimed in any previous claim, wherein said oxyacid salt contains an oxyacidic anion of an element selected from the group comprising B, Al, Si, Ge, Sn, Pb, As, Sb, Bi, Se, Te, P, Ti, Zr, V, Nb, Ta, Cr, Mo, W, Mn and Fe, said salt being added in a concentration of between 2 and 200 grams per liter of solution.

7. The process as claimed in any previous claim, wherein fine particles of pigmenting substances are added to produce a coating of a required colour.

8. The process as claimed in any previous claim, arranged to produce a pore-free coating, wherein the current flow is progressively reduced to stop coating.

9. A ceramically-coated metal article produced by the process as claimed in any previous claim.

10. An apparatus for the batch ceramic coating of articles made of a valve metal selected from the group consisting of aluminium, zirconium, titanium, hafnium and alloys of these metals, said apparatus comprising:
an electrolytic bath comprising an aqueous solution of an alkali metal hydroxide;
an electrode immersed in or containing the electrolyte liquid;
another electrode comprising at least one of said articles to be coated and means to suspend said article in said electrolyte;
a source of alternate electric current from a high voltage source of at least 700 V;
means for shaping the AC wave form, whereby shaped-wave electric current rises from zero to its maximum height and falls to below 40% of its maximum height within less than a quarter of a full alternating cycle;
connector elements to complete an electrochemical circuit, and
means for adding to said bath, while the apparatus is in operation, a controlled supply of an oxyacid salt of an alkali metal.

11. An apparatus as claimed in claim 10, wherein the high voltage source is a step-up transformer of up to 1,000 V and said means for shaping said AC waveform is a capacitor bank connected in series between said source and said valve metal.

12. An apparatus for the serial ceramic coating of articles made of a valve metal selected from the group consisting of aluminium, zirconium, titanium, hafnium and alloys of these metals, said apparatus comprising:
a first electrolytic bath comprising an aqueous solution of an alkali metal hydroxide;
a second electrolytic bath comprising an aqueous solution of an alkali metal hydroxide, and a low concentration of an oxyacid salt of an alkali metal;
a third electrolytic bath comprising an aqueous solution of an alkali metal hydroxide, and a higher concentration than is present m said second bath of an oxyacid salt of an alkali metal;
electrodes immersed in or containing the electrolyte liquids;
electrodes comprising at least one of said articles to be coated and means to suspend said article in said electrolytes;
means for transferring said articles from said first bath to said second bath and then to said third bath;
a source of AC electric potential of at least 700 V;
means for shaping the AC wave form, whereby shaped-wave electric current rises from zero to its maxium height and falls to below 40% of its maximum height within less than a quarter of a full alternating cycle; and
connector elements to complete an electrochemical circuit in each bath.

13. An apparatus as claimed in claim 12, wherein the high voltage source is a step-up transformer of up to 1,000 V and said means for shaping said AC waveform is a capacitor bank connected in series between said source and said valve metal.

## Patentansprüche

1. Verfahren zur Herstellung einer Keramikbeschichtung auf einem Ventilmetall, ausgewählt aus der Gruppe bestehend aus Aluminium, Zirkonium, Titan, Hafnium und Legierungen aus diesen Metallen, wobei das Verfahren aufweist:
das Eintauchen des Metalls als Elektrode in ein Elektrolytbad, welches eine wäßrige Lösung eines Alkalimetallhydroxids enthält;
das Bereitstellen einer Gegenelektrode, die in die Elektrolytflüssigkeit eingetaucht ist oder eine solche enthält;
das Hindurchleiten eines modifizierten, wellengeformten elektrischen Wechselstroms von einer Hochspannungsquelle mit mindestens 700 V durch eine Oberfläche des zu beschichtenden Metalls und die gegenüberliegende Elektrode, wobei der modifizierte, wellengeformte elektrische Strom von Null bis zur maximalen Stärke ansteigt und innerhalb von weniger als einem Viertel eines vollen Wechselzyklusses auf unter 40 % seiner maximalen Stärke abfällt, um dadurch einen Durchschlag, eine Erhitzung, ein Schmelzen und eine thermische Verdichtung eines Hydroxidfilms zu verursachen, der auf der Oberfläche des Metalls gebildet wird, um eine Keramikbeschichtung am Metall zu bilden und diese darauf zu verschweißen, und
das Ändern der Zusammensetzung des Elektrolyts während der Bildung der Keramikbeschichtung, wobei die Änderung durch die Zugabe eines Oxyacidsalzes eines Alkalimetalls bewirkt wird.

2. Verfahren nach Anspruch 1, wobei der modifizierte wellengeformte elektrische Strom durch die Verwendung eines zwischen der Hochspannungsquelle und dem Metall in Serie geschalteten Kondensatorblockes erhalten wird.

3. Verfahren nach Anspruch 1 oder Anspruch 2, wobei es sich bei dem hinzugefügten Salz um Natriumtetrasilicat handelt.

4. Verfahren nach einem der vorhergehenden Ansprüche, optimiert zur Schaffung einer größtmöglichen Haftkraft zwischen dem Metall und der Beschichtung, wobei das Elektrolyt im wesentlichen aus einer wäßrigen Lösung besteht, die zwischen 0,5 und 2 g/Liter Natriumhydroxid enthält.

5. Verfahren nach einem der vorhergehenden Ansprüche, optimiert zur Schaffung einer größtmöglichen Haftkraft zwischen dem Metall und der Beschichtung, wobei das Elektrolyt im wesentlichen aus einer wäßrigen Lösung besteht, die zwischen 0,5 und 2 Gramm Kaliumhydroxid pro Liter enthält.

6. Verfahren nach einem der vorhergehenden Ansprüche, wobei das Oxyacidsalz ein oxosaures Anion eines Elements, ausgewählt aus der Gruppe mit B, Al, Si, Ge, Sn, Pb, As, Sb, Bi, Se, Te, P, Ti, Zr, V, Nb, Ta, Cr, Mo, W, Mn und Fe, enthält, wobei das Salz in einer Konzentration von zwischen 2 und 200 Gramm pro Liter der Lösung hinzugefügt wird.

7. Verfahren nach einem der vorhergehenden Ansprüche, wobei feine Partikel pigmentierender Substanzen hinzugefügt werden, um eine Beschichtung einer erforderlichen Farbe zu erzeugen.

8. Verfahren nach einem der vorhergehenden Ansprüche, welches für die Erzeugung einer porenfreien Beschichtung ausgelegt ist, bei welchem der Stromfluß fortschreitend vermindert wird, um die Beschichtung zu stoppen.

9. Keramisch beschichteter Metallartikel, hergestellt durch den Prozeß gemäß einem der vorhergehenden Ansprüche.

10. Vorrichtung für die Großmengen-Keramikbeschichtung von Artikeln, hergestellt aus einem Ventilmetall, ausgewählt aus der Gruppe bestehend aus Aluminium, Zirkonium, Titan, Hafnium und Legierungen aus diesen Metallen, wobei die Vorrichtung aufweist:
ein Elektrolytbad, mit einer wäßrigen Lösung eines Alkalimetallhydroxids;
eine Elektrode, die in die Elektrolytflüssigkeit eingetaucht ist oder welche diese enthält;
eine weitere Elektrode, umfassend mindestens einen der zu beschichtenden Artikel, und ein Mittel, um den Artikel in den Elektrolyten zu hängen;
eine Wechselstromquelle von einer Hochspannungsquelle mit mindestens 700 V;
ein Mittel zur Formung der Wechselstromwellenform, wobei der wellengeformte elektrische Strom von Null bis zu seiner maximalen Höhe ansteigt und innerhalb von weniger als einem Viertel eines vollen Wechselzyklusses auf unter 40 % seiner maximalen Höhe abfällt;
Verbindungselemente, um einen elektrochemischen Kreislauf zu schließen; und
ein Mittel, um dem Bad, während die Vorrichtung in Betrieb ist, eine kontrollierte Menge eines Oxyacidsalzes eines Alkalimetalls hinzuzufügen.

11. Vorrichtung nach Anspruch 10, wobei es sich bei der Hochspannungsquelle um einen Aufwärtstransformator mit bis zu 1000 V handelt, und wobei es sich bei dem Mittel zur Formung der Wechselstromwellenform um einen Kondensatorblock handelt, der in Serie zwischen der Quelle und dem Ventilmetall geschaltet ist.

12. Vorrichtung für die serielle Keramikbeschichtung von Artikeln, hergestellt aus einem Ventilmetall, ausgewählt aus der Gruppe bestehend aus Aluminium, Zirkonium, Titan, Hafnium und Legierungen aus diesen Metallen, wobei die Vorrichtung umfaßt:
ein erstes Elektrolytbad mit einer wäßrigen Lösung eines Alkalimetallhydroxids;
ein zweites Elektrolytbad mit einer wäßrigen Lösung eines Alkalimetallhydroxids und einer geringen Konzentration eines Oxyacidsalzes eines Alkalimetalls;
ein drittes Elektrolytbad mit einer wäßrigen Lösung eines Alkalimetallhydroxids und einer höheren Konzentration eines Oxyacidsalzes eines Alkalimetalls als im zweiten Bad;
Elektroden, die in die Elektrolytflüssigkeit eingetaucht sind oder welche diese Flüssigkeit enthalten;
Elektroden, die mindestens einen der zu beschichtenden Artikel aufweisen, und ein Mittel, um den Artikel in die Elektrolyte zu hängen;
ein Mittel zum Übertragen der Artikel vom ersten Bad in das zweite Bad und danach in das dritte Bad;
eine Wechselstromquelle mit mindestens 700 V;
ein Mittel zur Formung der Wechselstromwellenform, wobei der wellengeformte elektrische Strom von Null bis zu seiner maximalen Höhe ansteigt und innerhalb von weniger als einem Viertel eines vollen Wechselzyklusses auf unter 40 % seiner maximalen Höhe abfällt; und
Steckerelemente, um einen elektrochemischen Kreislauf in jedem Bad zu schließen.

13. Vorrichtung nach Anspruch 12, wobei es sich bei der Hochspannungsquelle um einen Aufwärtstransformator von bis zu 1000 V handelt, und wobei es sich bei dem Mittel zum Formen der Wechselstromwellenform um einen Kondensatorblock handelt, der in Serie zwischen der Quelle und dem Ventilmetall angeschlossen ist.

## Revendications

1. Procédé de formation d'un revêtement céramique sur un métal pour soupape choisi dans le groupe constitué de l'aluminium, du zirconium, du titane, de l'hafnium et d'alliages de ces métaux, ledit procédé comprenant les étapes consistant :
à immerger ledit métal comme électrode dans un bain électrolytique comprenant une solution aqueuse d'un hydroxyde de métal alcalin,
à installer une électrode opposée immergée dans l'électrolyte liquide ou le contenant,
à faire passer un courant électrique alternatif à onde mise en forme modifiée d'une source de haute tension d'au moins 700 V à travers une surface dudit métal à revêtir et ladite électrode opposée, ledit courant électrique à onde mise en forme modifiée augmentant de zéro à sa valeur maximale et descendant en dessous de 40% de sa valeur maximale en moins d'un quart d'un cycle alternatif complet, provoquant ainsi un claquage diélectrique, le chauffage, la fusion et le compactage thermique d'une mince couche d'hydroxyde formée à la surface dudit métal pour former et souder un revêtement céramique sur ledit métal, et
à modifier la composition dudit électrolyte tandis que le revêtement céramique est en cours de formation, ladite modification s'effectuant en ajoutant un sel d'oxyacide d'un métal alcalin.

2. Procédé selon la revendication 1, dans lequel ledit courant électrique à onde mise en forme modifiée est obtenu en utilisant un bloc de condensateurs connectés en série entre ladite source de haute tension et ledit métal.

3. Procédé selon la revendication 1 ou 2, dans lequel ledit sel ajouté est le tétrasilicate de sodium.

4. Procédé selon l'une quelconque des revendications précédentes, optimisé pour assurer une adhérence maximale entre ledit métal et ledit revêtement, dans lequel ledit électrolyte est constitué essentiellement d'une solution aqueuse contenant 0,5-2 g/l d'hydroxyde de sodium.

5. Procédé selon l'une quelconque des revendications précédentes, optimisé assurer une adhérence maximale entre ledit métal et ledit revêtement, dans lequel ledit électrolyte est constitué essentiellement d'une solution aqueuse contenant 0,5-2 g/l d'hydroxyde de potassium.

6. Procédé selon l'une quelconque des revendications précédentes, dans lequel ledit sel d'oxyacide contient un anion oxyacide d'un élément choisi dans le groupe comprenant B, Al, Si, Ge, Sn, Pb, As, Sb, Bi, Se, Te, P, Ti, Zr, V, Nb, Ta, Cr, Mo, W, Mn et Fe, ledit sel étant ajouté en une concentration dans la plage de 2 à 200 grammes par litre de solution.

7. Procédé selon l'une quelconque des revendications précédentes, dans lequel de fines particules de substances pigmentaires sont ajoutées pour produire un revêtement d'une couleur requise.

8. Procédé selon l'une quelconque des revendications précédentes, aménagé pour produire un revêtement exempt de pores, dans lequel le flux de courant est progressivement réduit pour mettre fin au revêtement.

9. Article métallique revêtu de céramique produit par le procédé selon l'une quelconque des revendications précédentes.

10. Appareil pour le revêtement discontinu de céramique d'articles constitués d'un métal de soupape choisi dans le groupe constitué de l'aluminium, du zirconium, du titane, de l'hafnium et d'alliages de ces métaux, ledit appareil comprenant :
un bain électrolytique comprenant une solution aqueuse d'un hydroxyde de métal alcalin,
une électrode immergée dans l'électrolyte liquide ou le contenant,
une autre électrode comprenant au moins l'un desdits articles à revêtir et un moyen pour suspendre ledit article dans ledit électrolyte,
une source de courant électrique alternatif d'une source de haute tension d'au moins 700 V,
un moyen pour mettre en forme la forme d'onde CA par lequel le courant électrique à onde mise en forme augmente de zéro à sa valeur maximale et descende en dessous de 40% de sa valeur maximale en moins d'un quart d'un cycle alternatif complet,
des éléments de connexion pour parachever un circuit électrochimique, et
un moyen pour ajouter audit bain, pendant que l'appareil est en service, une quantité contrôlée d'un sel d'oxyacide d'un métal alcalin.

11. Appareil selon la revendication 10, dans lequel la source de haute tension est un transformateur élévateur de tension jusqu'à 1000 V et ledit moyen pour mettre en forme ladite forme d'onde CA est un bloc de condensateurs connectés en série entre ladite source à haute tension et ledit métal de soupape.

12. Appareil pour le revêtement céramique en série d'articles constitués d'un métal de soupape choisi dans le groupe constitué de l'aluminium, du zirconium, du titane, de l'hafnium et d'alliages de ces métaux, ledit appareil comprenant :
un premier bain électrolytique comprenant une solution aqueuse d'un hydroxyde de métal alcalin,
un deuxième bain électrolytique comprenant une solution aqueuse d'un hydroxyde de métal alcalin et une faible concentration d'un sel d'oxyacide d'un métal alcalin,
un troisième bain électrolytique comprenant une solution aqueuse d'un hydroxyde de métal alcalin et une concentration d'un sel d'oxyacide d'un métal alcalin supérieure à celle présente dans le deuxième bain,
des électrodes immergées dans les électrolytes liquides ou les contenant,
des électrodes comprenant au moins l'un desdits articles à revêtir et un moyen pour suspendre ledit article dans lesdits électrolytes,
un moyen de transfert desdits articles dudit premier bain audit deuxième bain et ensuite audit troisième bain,
une source de potentiel électrique CA d'au moins 700 V,
un moyen pour mettre en forme la forme d'onde CA par lequel le courant électrique à onde mise en forme augmente de zéro à sa valeur maximale et descende en dessous de 40% de sa valeur maximale en moins d'un quart d'un cycle alternatif complet, et
des éléments de connexion pour parachever un circuit électrochimique dans chaque bain.

13. Appareil selon la revendication 12, dans lequel la source de haute tension est un transformateur élévateur de tension jusqu'à 1000 V et ledit moyen de mise en forme de ladite forme d'onde CA est un bloc de condensateurs connectés en série entre ladite source de haute tension et ledit métal de soupape.
